



US005135671A

**United States Patent [19]****Kapuscinski et al.****[11] Patent Number: 5,135,671****[45] Date of Patent: Aug. 4, 1992**

[54] **MULTIFUNCTIONAL VISCOSITY INDEX IMPROVER CONTAINING UNITS FROM UNSATURATED CHLORIDES AND AROMATIC AMINES**

[75] Inventors: **Maria M. Kapuscinski, Carmel; Theodore E. Nalesnik, Wappingers Falls; Robert T. Biggs, Walden; Raymond C. Schlicht, Fishkill, all of N.Y.**

[73] Assignee: **Texaco Inc., White Plains, N.Y.**

[21] Appl. No.: **690,240**

[22] Filed: **Apr. 24, 1991**

[51] Int. Cl.<sup>5</sup> **C10M 149/12**

[52] U.S. Cl. **252/50; 525/331.7**

[58] Field of Search **525/292, 331.7, 382; 252/50**

[56]

**References Cited****U.S. PATENT DOCUMENTS**

|           |         |             |           |
|-----------|---------|-------------|-----------|
| 4,160,739 | 7/1979  | Stambaugh   | 252/50    |
| 4,816,172 | 3/1989  | Kapuscinski | 252/47.5  |
| 4,886,611 | 12/1989 | Kapuscinski | 252/50    |
| 5,021,177 | 6/1991  | Kapuscinski | 525/331.7 |
| 5,030,695 | 7/1991  | Cozewith    | 525/331.7 |
| 5,075,383 | 12/1991 | Migdal      | 252/50    |

*Primary Examiner*—Willis, Jr. Prince

*Assistant Examiner*—Thomas Steinberg

*Attorney, Agent, or Firm*—Robert A. Kulason; James J. O'Loughlin; Vincent A. Mallare

[57] **ABSTRACT**

Multifunctional viscosity index improvers for lubricating oils containing olefin copolymers which have pendant groups derived from vinylbenzyl chloride and N-phenyl-p-phenylene diamine.

**3 Claims, No Drawings**

**MULTIFUNCTIONAL VISCOSITY INDEX  
IMPROVER CONTAINING UNITS FROM  
UNSATURATED CHLORIDES AND AROMATIC  
AMINES**

**BACKGROUND OF THE INVENTION**

This invention relates to a novel multi-functional lubricant additive which is a dispersant, antioxidant and antiwear VI improver additive when employed in a lubricating oil composition.

It is well known to those skilled in the art that hydrocarbon lubricating oils must be formulated by addition of various additives to improve their properties.

In the case of lubricating oils, typified by those employed in railway, automotive, aircraft, marine, etc., service, it is found that they become degraded during use due inter alia to formation of sludge which may be generated by deterioration of the oil or by introduction of undesirable components from other sources including the fuel or the combustion air. In order to maintain and improve the properties of the lubricating oil, various additives have heretofore been provided; and these have been intended to improve the viscosity index, dispersancy, oxidative stability, antiwear properties, etc.

It is, therefore, an object of this invention to provide an additive system which imparts to lubricating oils these improved properties of viscosity index, dispersancy, antiwear properties and oxidative stability. Other objects will be apparent to those skilled in the art.

**DISCLOSURE STATEMENT**

The art contains many teachings on the use of polymer additives in lubricating oil compositions. Ethylene-propylene copolymers and ethylene-propylene-diene terpolymers which have been further derivatized to provide multifunctional properties in lubricating oil compositions illustrate this polymer type of oil additive.

U.S. Pat. No. 3,522,180 discloses a method for the preparation of an ethylene-propylene copolymer substrate effective as a viscosity index improver for lubricating oils.

U.S. Pat. No. 4,089,794 discloses ethylene copolymers derived from ethylene and one or more (C<sub>3</sub> to C<sub>28</sub>) alpha-olefin solution grafted with an ethylenically-unsaturated carboxylic acid material followed by a reaction with a polyfunctional material reactive with carboxyl groups, such as a polyamine, a polyol, or a hydroxylamine, which reaction product is useful as a sludge and varnish control additive in lubricating oils.

U.S. Pat. No. 4,137,185 discloses a stabilized imide graft of an ethylene copolymer additive for lubricants.

U.S. Pat. No. 4,146,489 discloses a graft copolymer where the backbone polymer is an oil-soluble ethylene-propylene copolymer or an ethylene-propylene-diene modified terpolymer with a graft monomer of C-vinyl-pyridine or N-vinylpyrrolidone to provide a dispersant VI improver for lubricating oils.

U.S. Pat. No. 4,820,776 discloses lubricants and fuel oils of improved properties containing ethylene-propylene copolymer derived with N-vinyl pyrrolidone and phenothiazine.

U.S. Pat. No. 4,320,019 discloses a multipurpose lubricating additive prepared by the reaction of an interpolymer of ethylene and a (C<sub>3</sub>-C<sub>8</sub>) alpha-monoolefin with an olefinic carboxylic acid acylating agent to form

an acylating reaction intermediate which is then reacted with an amine.

U.S. Pat. No. 4,764,304 discloses a lubricating oil dispersant VI improver composition containing an additive prepared by the reaction of an olefin copolymer and an unsaturated isocyanate to form reactive intermediate which is then reacted with heterocyclic amines.

U.S. Pat. No. 4,340,689 discloses a process for grafting a functional organic group onto an ethylene copolymer or an ethylene-propylene-diene terpolymer.

U.S. Pat. No. 4,357,250 discloses a reaction product of a copolymer an olefin carboxylic acid via the "ene" reaction followed by a reaction with a monoamine-polyamine mixture.

U.S. Pat. No. 4,382,007 discloses a dispersant—VI improver prepared by reacting a polyamine-derived dispersant with an oxidized ethylene-propylene polymer or an ethylene-propylene diene terpolymer.

U.S. Pat. No. 4,144,181 discloses polymer additives for fuels and lubricants comprising a grafted ethylene copolymer reacted with a polyamine, polyol or hydroxylamine and finally reacted with an alkaryl sulfonic acid.

The disclosures in the foregoing patents which relate to VI improvers and dispersants for lubricating oils; namely, U.S. Pat. Nos. 3,522,180, 4,026,809, 4,089,794, 4,137,185, 4,144,181, 4,146,489, 4,820,776, 4,320,019, 4,340,689, 4,357,250, and 4,382,007 are incorporated herein by reference.

An object of this invention is to provide a novel derivatized polymer composition which imparts viscosity index improving, dispersant, antiwear and antioxidant activity to lubricating oil compositions.

Another object is to provide a process for preparing a copolymer derivatized with an unsaturated chloride to form a reactive intermediate which is then reacted with an antioxidant aromatic hindered amine.

Still another object is to provide a process for preparing a copolymer derivatized with graft monomers formed from a reactive unsaturated chloride and aromatic hindered amine to yield a modified copolymer which performs as a viscosity index improver, dispersant, antiwear agent and antioxidant in lubricating oil.

Also another object is to provide a multi-functional lubricant additive effective for imparting viscosity index, dispersant, antiwear and antioxidant properties to a lubricating oil composition.

**SUMMARY OF THE INVENTION**

The present invention is directed to multi-functional VI improvers based on polymer prepared in one step by free-radical grafting of monomer derived from unsaturated chloride and aromatic hindered amine onto olefin copolymers being a polymer base.

Also, the present invention is directed to multifunctional VI improvers based on a polymer prepared in a two-step process which comprises using olefin copolymers as a polymer base derived with unsaturated chlorides and hindered aromatic amines. First, unsaturated 60 chloride is grafted under elevated temperatures with the addition of a free radical initiator. The grafting reaction is followed by a capping of a hindered aromatic amine.

The reaction product of the present invention preferably is prepared using ethylene-propylene copolymer (EPM) or ethylene-propylene diene terpolymer (EPDM) as a polymer base, a vinylbenzyl chloride and N-phenyl-p-phenylene diamine as modifying agents.

The lubricant additive of the present invention comprises an oil of lubricating viscosity and an effective amount of the novel reaction product. The lubricating oil will be characterized by having viscosity index improver, dispersancy, antiwear and antioxidant properties. The methods of preparation are also contemplated.

#### DETAILED DESCRIPTION OF THE INVENTION

This invention, as discussed briefly above, is directed to a polymer comprising an oil-soluble, substantially linear, carbon-carbon backbone polymer bearing functional units thereon, derived from an unsaturated monomer containing chlorine group such as vinyl benzyl chlorine and hindered aromatic amine such as N-phenyl-p-phenylene diamine.

The charge polymer which may be employed in the practice of the present process of this invention may include an oil-soluble, substantially linear, carbon-carbon backbone polymer. Typical carbon-carbon backbone polymers, prepared from monomers bearing an ethylenically unsaturated polymerizable double bond, which may be employed include homopolymers or copolymers prepared from a monomer containing the grouping:



wherein A may be a hydrogen, hydrocarbon such as alkyl, aryl (particularly phenyl) etc., —OOCR typified by acetate or less preferred acyloxy (typified by —OOCR), halide, epoxy, benzyl, etc. R'' may be divalent hydrocarbon typified alkylene, alkarylene, cycloalkylene, arylene, etc.

The polymer or copolymer substrate employed in the novel additive of the invention may be prepared from ethylene and propylene or it may be prepared from ethylene and a higher olefin within the range of C<sub>3</sub> to C<sub>10</sub> alpha-monoolefins. The polymer or copolymer substrate may also be prepared from isoprene, styrene or butadiene.

More complex polymer substrates often designated as interpolymers may be prepared using a third component. The third component generally used to prepare an interpolymer substrate is a polyene monomer selected from non-conjugated dienes and trienes. The non-conjugated diene component is one having from 5 to 14 carbon atoms in the chain. Preferably, the diene monomer is characterized by the presence of a vinyl group in its structure and can include cyclic and bicyclo compounds. Representative dienes include 1,4-hexadiene, 1,4-cyclohexadiene, dicyclopentadiene, 5-ethylidene-2-norbornene, vinylnorbornene, 5-methylene-2-norbornene, 1,5-heptadiene, and 1,6-octadiene. A mixture of more than one diene can be used in the preparation of the interpolymer. A preferred non-conjugated diene for preparing a terpolymer or interpolymer substrate is 5-ethylidene-2-norbornene.

The polymer and copolymers prepared from the above-mentioned monomers having short and long branches or star shape structure may also be employed.

The preferred carbon-carbon backbone polymers include those selected from the group consisting of ethylene-propylene copolymers (EPM or EPR) and ethylene-propylene-diene terpolymers (EPDM or EPT).

When the charge polymer is an ethylene-propylene copolymer (EPM), it may be formed by copolymerization of ethylene and propylene under known conditions, preferably Ziegler-Natta reaction conditions. The preferred EPM copolymers contain units derived from the ethylene in amount of 40-90 mole %, preferably 55-80 mole %, say 59 mole %, the remainder being derived from propylene.

The molecular weight  $\bar{M}_n$  of the EPM copolymers which may be employed may be about 5,000 to about 1,000,000, preferably about 20,000 to about 200,000, and most preferably about 80,000. The molecular weight distribution may be characterized by  $M_w/M_n$  of less than about 15, preferably 1.2-10, say 1.8.

When the charge polymer is ethylene-propylenediene terpolymer (EPT or EPDM), it may be formed by copolymerization of ethylene, propylene, and diene monomers. The diene monomer is commonly a non-conjugated diene typified by dicyclopentadiene; 1,4-hexadiene; ethylidene norbornene or vinyl norbornene. Polymerization is effected under known conditions generally comparable to those employed in preparing the EPM products. The preferred terpolymers contain units derived from ethylene in amount of 40-90 mole %, preferably 50-65 mole %, say 59 mole % and units derived from propylene in an amount of 20-60 mole %, preferably 30-50 mole %, say 41 mole % and units derived from diene third monomer in amount of 0.1-15 wt %, preferably 0.1-3 wt %, say 0.3 wt %. The molecular weight  $\bar{M}_n$  of the terpolymers may typically be about 5,000 to about 500,000, preferably about 20,000 to about 200,000 and most preferably about 80,000. Molecular weight distribution of the useful polymers is preferably narrow viz a  $M_w/M_n$  of typically less than 10, preferably 1.5-5, say about 2.2.

According to the process of this invention, the additive may be prepared in a one-step or two-step procedure. In one step process, a functional monomer derived from such unsaturated chloride as vinyl benzyl chloride (VBC) or croton chloride (CC) and aromatic amine such as N-phenyl-phenylene diamine (NPPDA) is grafted onto polymer. In two-step process unsaturated chloride is grafted first followed by capping of the amine. The two processes are described, respectively, below.

#### ONE-STEP PROCESS

In the one-step process, a monomer derived from unsaturated chloride such as vinyl benzyl chloride (VBC), and aromatic amine such as N-phenyl-phenylene diamine (NPPDA) is grafted onto polymer.

##### 1. Preparation of Grafting Monomers



where:

R<sub>1</sub> is an organic linear, cyclic or heterocyclic, and aromatic or heteroaromatic unit composed of hydrocarbon and/or contain one or more atom of oxygen, nitrogen, sulfur or phosphorus.

R<sub>2</sub> is an organic linear cyclic or heterocyclic, and aromatic group composed of hydrocarbon and/or contain one or more atoms of oxygen, nitrogen, sulfur or phosphorus.

R<sub>3</sub> is a hydrogen or R<sub>2</sub>

## 2. Grafting Reaction



where P is a carbon-carbon polymer

## TWO-STEP PROCESS

In the two-step process unsaturated chloride is grafted onto the carbon-carbon polymer under elevated temperatures with addition of a free radical initiator. The grafting reaction is followed by capping of amine. The following reactions illustrate the process of the invention:

## 1. Grafting Reaction



## 2. Capping Reaction



where P, R<sub>1</sub>, R<sub>2</sub> and R<sub>3</sub> are as defined above for the one step reaction.

It is a feature of the process of this invention that the graft monomer may be grafted onto carbon-carbon backbone polymers in the presence of a free radical initiator.

Any of the typical free radical initiators, such as dicumyl peroxide, 2,2'Azobis(2-methyl-N-[1,1-bis(hydroxymethyl)ethyl]propionamide, di-tert-butylperoxide, azobisisobutyronitrile, diacetylperoxide, and diisopropylperoxidicarbonate may be employed in this process.

The reaction product of the present invention preferably is prepared using such materials as:

vinyl benzyl chloride

crotonyl chloride

3-chloro-2-methyl propene

and an amine, such as N-phenyl p-phenylenediamine

In the practice of the process of this invention, 100 weight parts of charge EPM or EPT may be added to 100-1000 weight parts, say 300-60 weight parts of diluent-solvent. Typical diluent-solvent may be a hydrocarbon solvent such as mineral oil, n-hexane, n-heptane, or tetrahydrofuran. Preferred solvent may be a commercial hexane containing principally hexane isomers or a commercial mineral grafting oil. Reaction mixture may then be heated under nitrogen to reaction conditions of 60° C.-180° C., preferably 150° C.-170° C., say 155° C. When n-hexane or other low boiling solvent is used, reaction is carried out in pressure reactor at 15-300 psig, preferably 180-200 psig, say 200 psig.

In the grafting reaction of the one-step process, a graft monomer typically prepared from vinylbenzyl chloride and N-phenyl-p-phenylenediamine, is admitted in an amount of about 1-20 weight parts, preferably 3 to 8 weight parts. There is also added a free radical initiator in solution in grafting solvent. Typical free radical initiators may include dicumyl peroxide, or di-tert-butyl peroxide. The solvent is preferably the same as that in which the EPM or EPT is dissolved. The initiator may be added in an amount of 0.2-20 weight parts,

preferably 1.5 to 4.0 weight parts. The preferred free radical initiator is a dicumyl peroxide (DICUP).

The reaction is carried out at a temperature at least as high as the decomposition temperature of the initiator, typically 150° C.-160° C. or higher for the time needed for bonding the graft reactive monomer onto the base EPM or EPT polymer.

In the two-step process, the grafting reaction is performed as described above except that unsaturated chloride such as vinylbenzyl chloride instead of a functional monomer containing aromatic amine is charged. When grafting reaction is completed, amidization reaction is performed.

Amidization may be carried out by adding the graft polymer containing chlorine groups to a reaction vessel together with inert-diluent solvent. In the preferred embodiment, reaction may be carried out in the same solvent and in the same reaction medium as that in which the polymer is dissolved.

In carrying out the present process, the graft polymer bearing pendant chloride groups may be reacted with an aromatic amine containing at least one non-tertiary nitrogen atom.

An amine, typically N-phenyl-p-phenylenediamine is added to the reaction vessel. The amount of amine added is preferably 0.1-5 moles, say 1.2 moles per mole of chlorine compound charged during the first step.

The amidization reaction is carried out over 0.1-10 hours, preferably 2-4 hours at 100°-180° C., say 155° C. with agitation.

The product graft polymer may be characterized by the presence of pendant reactive groups containing aromatic amine bonded to the polymer backbone through the residue of the unsaturated chloride, the latter being bonded to the polymer backbone through one of the carbon atoms which formed the ethylenically unsaturated double bond.

Typically, the graft product polymer may contain 0.05-10 units derived from graft monomer and amine per 1000 carbon atoms of the charge backbone polymer.

For ease of handling, enough mineral oil, such as SUS 100 oil typified by SNO-100 is then added to obtain a fluid concentrate product at room temperature. The product is typically obtained as a solution of about 4 to about 20 parts in about 80 to about 96 parts of oil. When the grafting reaction is carried out in hexane (or other low boiling solvent), a stripping step is included.

The fluid solution (a lubricating additive) is used for further testing.

It is a feature of this invention that the so-prepared polymer solution in oil may find use in lubricating oils as multi-functional additive (e.g., dispersant viscosity index improvers which provide antiwear and antioxidant properties, etc.) when present in effect amount of about 1.0 to about 20 wt %, preferably 3-15 wt %, preferably about 9 wt %.

Lubricating oils in which the multi-functional additives of this invention may find use may include automotive, aircraft, marine, railway, etc., oils; oils used in spark ignition or compression ignition; summer or winter oils, etc. Typically, the lubricating oils may be characterized by a b.p. of about 570° F. to about 660° F., preferably 610° F.; an e.p. of about 750° F. to about 1200° F., preferably 1020° F.; an API gravity of about 25 to about 31, preferably about 29.

A typical lubricating oil in which the polymer of this invention may be present may be a standard SAE

5W-30 hydrocarbon motor oil formulation having the composition as set forth below in Table 1.

TABLE 1

|                                                                      | Wt % |
|----------------------------------------------------------------------|------|
| Base Oil                                                             | 82   |
| Viscosity Index Improver<br>(additive of this invention)             | 9    |
| (10 w % ethylene-propylene copolymer<br>in 90% inert oil)            |      |
| Standard Additive Package:                                           | 9    |
| polysisobutyl (M1290) <sub>n</sub> succinimide<br>(dispersant)       |      |
| calcium sulfonate (detergent)                                        |      |
| zinc diethiophosphate (antiwear)                                     |      |
| di-nonyl diphenyl amine (antioxidant)                                |      |
| 4,4'-methylene-bis (2,6-di- <i>t</i> -butyl phenol)<br>(antioxidant) |      |

Use of the additive of this invention makes it possible to readily increase the viscosity index by 25-40 units, say 35 units, and to obtain improved ratings on the tests measuring the dispersancy of the system. The viscosity index is determined by ASTM Test D-445.

The present invention comprises making dispersant, antiwear and antioxidant VI improvers by derivatizing hydrocarbon polymers such as ethylene-propylene copolymer (EPM) or ethylene-propylene-diene terpolymer (EPDM) with, pendant units containing hindered aromatic amine.

Addition of the above invention additives to a lubricating oil may be facilitated by use of a concentrate containing about 1 to about 20 wt %, preferably about 4 to about 14 wt % of polymer.

The tests and analysis used, according to the present invention, are provided below.

#### TESTS AND ANALYSIS

##### 1. Oxidation Stability

The antioxidant activity of the new multi-functional VI improver was examined by a proprietary test called the Bench Oxidation Test (BOT). In this test, the polymer solution is diluted with SNO-130 oil. The mixture is heated with stirring and air agitation. Samples are withdrawn periodically for analysis, by differential infrared analysis (DIR) to observe changes in the intensity of the carbonyl vibration band at 1710 cm<sup>-1</sup>. Higher carbonyl group intensity indicates a lower thermal oxidative stability of the sample. The result reported, as oxidation index, indicates the change in the intensity of the carbonyl vibration band at 1710 cm<sup>-1</sup> after 144 hours of oxidation. A lower rating indicates better thermal oxidative stability of the mixture.

##### 2. Dispersancy

The sample is blended into a formulated oil, not containing a dispersant, to form 10.0 wt % viscosity index improver solution. That blend is tested for dispersancy in the prototype VE Test. In this test, the turbidity of an oil containing an additive is measured after heating the test oil to which has been added a standard blow-by. The result correlates with dispersancy and is compared to three standards (excellent, good, fair) tested simultaneously with the test sample. The numerical rating decreases with an increase in dispersant effectiveness.

##### 3. Antiwear Properties

Antiwear performance of a new VI improver was determined by a Four-Ball Test (NMS-82-79, ASTM D-2266, ASTM4172). The VI improver solutions in

formulated oil, having Kinematic Viscosity at 100° C. around 16 cSt were evaluated.

In this test, four balls are arranged in an equilateral tetrahedron. The lower three balls are clamped securely in a test cup filled with lubricant and the upper ball held by a chuck which is motor driven, causing the upper ball to rotate against the fixed lower balls. Load is applied in an upward direction through a weight/lever arm system. Heaters allow operation at elevated oil temperatures. The test speeds available for each tester are 600 rpm, 1200 rpm, and 1800 rpm. Results are reported as average scar diameter (mm).

The amount of hindered aromatic amine incorporated onto OCP in the grafting process is determined by IR-analysis of isolated rubber. The amount of aromatic amine on the polymer is determined by aromatic stretch at 1600 cm<sup>-1</sup>. The rubber is isolated from solution by multiple precipitation using cyclohexane as a solvent and acetone as precipitator. The rubber (isolated as a solid) is dried in vacuum at 60° C. for 36 hours.

#### DESCRIPTION OF THE PREFERRED EMBODIMENTS

The practice of the process of this invention will be more apparent to those skilled in the art from the following examples wherein, as elsewhere in this specification, all parts are parts by weight unless otherwise set forth. Control examples are designated by an asterisk\*.

##### EXAMPLE I

In this example, a monomer was prepared from vinyl benzyl chloride (VBC) and N-phenyl-p-phenylenediamine (NPPDA).

18.42g (0.1 mole) of NPPDA is dissolved in 190 ml THF and mixed with 67.02 (1.2 mole) of calcium oxide. Then 15.62 g (0.1 mole) of VBC is added dropwise and mixture is heated at 70°-80° C. for 2 hours. Solid calcium chloride is removed by ultra-centrifugation and THF is distilled of under vacuum using a rotovapor. The product is used as it is for grafting reaction.

##### EXAMPLE II

The monomer prepared as described in Example 1 is grafted onto EPM containing around 0.3 mole % of vinyl norbornene in the presence of free radical initiator, dicumyl peroxide. EPM (Mn = 80,000 as measured by SEC) containing approximately 60 mole % of ethylene is used

100 w. parts of EPM dissolved in 210 parts of mineral grafting oil (SN-130) is heated to 155° C. (with stirring under nitrogen). 6.0 w. parts of monomer of Example 1 in 3.0 w. parts of grafting oil is added followed by 2.24 wt parts dicumyl peroxide dissolved in 6 wt parts of oil. The mixture is stirred using above conditions for 2 hours.

Then, the solvent neutral oil (SNO-100) is added to give a solution containing 13.0 wt % polymer. This solution is used for further testing.

##### EXAMPLE III

In this Example, 100 w parts of EPM dissolved in 210 parts of mineral grafting oil (SN-130) is heated to 155° C. (with stirring under nitrogen). 4.0 w parts of VBC in 3.0 w parts of grafting oil is added followed by 1.48 wt. parts dicumyl peroxide dissolved in 5 wt. parts of oil. The mixture is stirred using above conditions for 2 hours. Then, 5.8 wt. parts of NPPDA is added and the

reaction mixture is stirred and heated at 155°-165° C. for 2 hours.

Then, the solvent neutral oil (SNO-100) is added to give a solution containing 13.0 wt % polymer. This 5 solution is used for further testing.

#### EXAMPLE IV\*

In this example, 13.0 wt. % EPM solution in mineral oil is prepared. 100 wt parts of EPM which is used in the Example 1, is added to 218 wt. parts of SN-130 and 10 451.2 wr parts of SNO-100. The mixture is heated to 155° C. with stirring and under nitrogen for 3 hours until the rubber is completely dissolved.

#### RESULTS

The evaluation data for the samples of Examples II, III, and IV\* are listed below in Table 2. The sample numbers are related to the example numbers.

As seen below in Table 2, samples of Examples II and III containing units derived from vinyl benzyl chloride and NPPDA showed good antioxidant and dispersant or antiwear properties. By contrast, the reference sample IV\* which contains unmodified EPM did not give any antiwear, dispersancy or antioxidant performance.

The above data indicate that EPM or EPDM copolymers containing pendant units derived from vinyl benzyl chloride and N-phenyl-p-phenylene diamine form multi-functional VI improvers exhibiting dispersant, antiwear and antioxidant performance in motor oils.

TABLE 2

| SAMPLE                    | Properties of VI Improvers |     |     |
|---------------------------|----------------------------|-----|-----|
|                           | II                         | III | IV* |
| <u>MATERIAL wt. parts</u> |                            |     |     |

TABLE 2-continued

| SAMPLE                      | Properties of VI Improvers |          |       |
|-----------------------------|----------------------------|----------|-------|
|                             | II                         | III      | IV*   |
| EPM (0.3 diene)             | 100                        | 100      | 100   |
| Monomer VBC-NPPDA           | 6.0                        | —        | —     |
| <u>Monomer</u>              |                            |          |       |
| VBC                         | —                          | 6.0      | —     |
| NPPDA                       | —                          | 5.8      | —     |
| DICUP                       | 2.24                       | 1.48     | —     |
| Grafting Oil                | 219.0                      | 218.0    | 218.0 |
| Diluent Oil                 | 442.0                      | 443.0    | 451.2 |
| OXIDATION INDEX(1)          | 0.0                        | 1.8      | 19.0  |
| ANTIWEAR PROPERTIES mm(2)   | 0.39                       | 0.6      | 1.7   |
| <u>BENCH DISPERSANCY(3)</u> |                            |          |       |
| Result                      | 44.7                       | 104      | 200   |
| Standards                   |                            | 33/59/99 |       |

(1) Change in the intensity of the carbonyl group IR vibration at 1710  $\text{cm}^{-1}$  after 144 hours in BOT.

(2) Four Ball Wear Test: 1800 rpm, 200° F., 40 kg, 2 hrs. 15W-40 formulation.

(3) As measured by Prototype Bench VE Test

20 We claim:

1. A lubricating oil composition comprising a major portion of lubricating oil and a minor effective viscosity index improving portion of a substantially linear graft polymer containing a substantially linear carbon-carbon backbone polymer and graft polymerized thereon, under nitrogen at a temperature ranging from about 60° C. to about 180° C. and a pressure ranging from about 15 to about 300 psig in the presence of free radical initiator, graft monomer of vinylbenzyl chloride which after 25 graft polymerization has been effected, having been amidized by reaction with N-phenyl-p-phenylene diamine.

2. The lubricating oil composition of claim 1 wherein said backbone polymer is a copolymer of ethylene-propylene or a terpolymer of ethylene-propylene-diene.

3. The lubricating oil additive of claim 1 wherein said minor effective viscosity index improving portion of said graft polymers is 0.1-20 wt % based on oil composition.

\* \* \* \* \*

40

45

50

55

60

65